

# United States Patent Office

2,761,795

Patented Sept. 4, 1956

1

2,761,795

## METHOD OF SOFTENING TEXTILE MATERIAL AND RESULTING PRODUCT

Joseph J. Carnes, Greenwich, Conn., assignor to American Cyanamid Company, New York, N. Y., a corporation of Maine

No Drawing. Application April 6, 1953,  
Serial No. 347,169

4 Claims. (Cl. 117—139.5)

This invention relates to a class of polymeric compounds which have outstanding characteristics as non-yellowing softening agents for cotton and rayon textiles during hot-finishing treatments and subsequent storage thereof. More particularly, the invention relates to a class of sulfosuccinic acid polyesters of either dihydroxyalkylamides or ethylene oxide condensation products thereof possessing softening properties, heat stability and other desirable characteristics.

In the course of their manufacture and finishing, cotton and rayon textiles are usually subjected to various heat treatments. Often, the textiles are treated with filters such as starch, gum tragacanth, gum ghatti, dextrines, and the like, in order to impart body to the cloth. These treatments, however, often result in the production of a relatively stiff fabric which is harsh-feeling and less desirable commercially than fabrics having a soft hand.

Consequently, the industry has resorted to the use of several types of compounds for the softening of the finished fabric and, in the case of rayon textiles, for imparting increased lubricity thereto. Among the compounds employed by the art have been sulfonated hydrocarbons, waxes, stearates, sulfated oils, such as cottonseed oil, peanut oil, and similar sulfonated or sulfated oil products. In view of the economics involved in textile manufacture, some of the most widely-employed softening agents have been sulfated and/or sulfonated tallow, sulfated and/or sulfonated mono- and diglycerides of tallow, cottonseed oil, coconut oil and others containing the relatively long carbon chain fatty acids.

However, the incorporation of even small amounts of these agents in cotton and rayon textiles has frequently resulted in the undesirable yellowing of the fabric subsequent to the finishing thereof. This is primarily due to the fact that the washed and/or sized fabric is ordinarily dried at temperatures of about 250—400° F. and is then immediately rolled into bolts. The inner layers of the bolted cloth retain the heat for a period of several days during which time these sulfated or sulfonated softening agents, all of which are relatively sensitive to heat, deteriorate sufficiently to cause serious yellowing of the treated fabric. Similarly, in the fabrication of garments from the treated textile materials, the cloth is frequently subjected to hot-pressing operations which cause these softening agents to deteriorate. Therefore, although sulfated and sulfonated fatty acids and fatty acid glycerides are recognized as acceptable textile softening agents, their lack of heat stability has rendered them undesirable for many textile finishing operations.

A principal purpose of the present invention is to provide a heat-stable, non-yellowing softening agent for cotton and rayon textiles during hot-finishing treatments and during subsequent storage thereof.

Other purposes, as well as features and advantages, of the present invention will become apparent from a consideration of the following specification wherein I have set forth a preferred embodiment of my inventive

2

concept which is to be considered illustrative but not limitative of my invention.

I have discovered that the members of a new class of polyesters of sulfosuccinic acid, and either dihydroxyalkylamides or ethylene oxide condensation products of such amides, possess outstanding textile softening properties without any appreciable tendency either to deteriorate under the influence of heat, or to cause any shade changes in the fabrics to which they are applied. In addition to these desirable qualities, this class of polymeric compounds has also been found to plasticize the starch sizes employed by the textile industry. Thus, the novel class of compounds of this invention provides the textile industry with a dual-purpose agent which acts both as a non-yellowing textile softening compound and a plasticizer for starch-sized fabrics.

A further important advantage of the invention resides in the fact that substantially all of the starting materials of these polyesters of sulfosuccinic acid are readily available commercially at relatively low cost, which renders the agents obtained extremely attractive to the manufacturers of textiles.

The novel class of heat-stable, non-yellowing textile softening agents of the invention has the following general polymeric formula:



wherein Me is a salt-forming cation, derived from any of the alkali metals, ammonium or other bases;  $n$  is the degree of polymerization and is an integer from 2 to about 12; and R is the residue of a dihydroxyalkylamide or an ethylene oxide condensation product thereof.

In order to define more properly the scope of the term "residue" of a dihydroxyalkylamide, the following generic structural formula is given as illustrative of the dihydroxyalkylamides from which the residues are derived by removal of the two hydroxy radicals. The formula is:



wherein  $\text{R}_1$  is an alkyl or alkenyl radical having from about 5 to about 22 carbon atoms;  $\text{R}_2$  is hydroxyalkyl or hydrogen; and  $\text{R}_3$  is hydroxyalkyl when  $\text{R}_2$  is hydroxyalkyl and is dihydroxyalkyl when  $\text{R}_2$  is hydrogen.

A consideration of the preceding definition therefore reveals the community of properties existing due to the presence in the dihydroxyalkylamide of an alkyl- or alkenyl-substituted amide group  $\text{RCON=}$  and two hydroxy groups capable of condensing in the linear polymerization to be described hereinafter.

Briefly, the polyesters of the present invention are prepared by reacting a fatty acid with a suitable dihydroxyalkylamine to obtain the corresponding dihydroxyalkylamide. This amide is then polyesterified by heating under the proper temperature and pressure conditions for the required period of time with maleic anhydride (or its equivalent such as maleic acid or fumaric acid) to form the polymaleate of the amide. This polymeric esterification is continued under the required reaction conditions until the desired or necessary number of ester units have united. The polymaleate is then sulfonated to form the polysulfosuccinate of the dihydroxyalkylamide. Preferably, the sulfonation is carried out by heating the polyester with an aqueous solution of an alkali metal or ammonium bisulfite or metabisulfite to obtain the corresponding salt. Salts of other bases may be obtained readily by first acidifying an alcoholic solution of the alkali metal or ammonium salt, whereby the free polyester of the sul-

fosuccinic acid is obtained, filtering off the inorganic salt of the acid used and reacting the free polyester with the desired base. Although they are not ordinarily employed in textile finishing treatments, salts of the polyvalent metals such as calcium, barium, zinc, lead, cadmium, and the like may be prepared, if desired, by adding stoichiometric quantities of their oxides or hydroxides to the alcoholic polymeric ester solution, followed by stirring until the salt formation is complete. Salts of organic bases such as methyl, ethyl, or butyl amine; guanylures; guanidine; hydroxyethylguanidine; biguanide; ethanolamine; triethanolamine; or higher aliphatic amines; aromatic amines; and heterocyclic bases such as nicotine, pyridine, quinoline, and alkaloids may be prepared by this method, as well as by direct sulfonation employing the sulfites and bisulfites of the organic bases.

In general, the polyesters of sulfosuccinic acid range from viscous liquids to hard waxy compositions depend-



ing on the number of ester units present and, to some extent, on the particular fatty acids and amines employed. It has been found that polymers containing from 2 to about 12 ester units possess the desirable textile softening characteristics. All of these products are dispersible in water and some of them are also soluble in hydrocarbon solvents. The corresponding monomeric sulfosuccinates (in which "n" would be 1) are generally unsatisfactory as textile softeners due to their heat instability, whereas the corresponding polyesters containing in excess of an average of 12 ester units are generally insufficiently dispersible or soluble to permit their use in textile treatments.

A convenient method of following the course of the polymerization reaction and the value of "n" exists in the determination of the acid number of the polyester, as expressed in ml. of KOH required to exactly neutralize 1 g. of product. The acid number decreases as the polymerization progresses. For example, an acid number of about 40 will indicate that the product contains an average ester unit content of about 1.5 to about 2, while an acid number of about 25-10 indicates an average ester unit content of 6 to 10, depending on the molecular weight of the dihydroxylalkylamide employed.

The fatty acids which have been found suitable for preparing the products of the present invention have the general formula  $R_1COOH$  wherein  $R_1$  represents an alkyl or alkenyl radical in which the number of carbon atoms is limited only by the commercial availability and cost of the particular fatty acid. The preferred range for the fatty acids applicable for the textile purposes of the present invention has been established to be from about 5 or 7 carbon atoms up to about 18 or 22 carbon atoms, although fatty acids having more or less carbon atoms are also suitable. Representative acids would include: stearic acid, lauric acid, palmitic acid, myristic acid, capric acid, behenic acid, arachidic acid, caprylic acid, caproic acid, valeric acid, butyric acid or other saturated fatty acids; oleic acid, ricinoleic acid, palmitoleic acid, pentenic acids, hexenic acids, sorbic acid, linoleic acid, decylenic acid, dodecylenic acid, or other unsaturated fatty acids.

Among the dihydroxyalkylamines suitable for reacting with the above-mentioned fatty acids are: diethanolamine; a-glycerol amine; b-glycerol amine; diisopropanolamine; dipropanolamine; etc.

The fatty acid and the dihydroxyalkylamine may be reacted in substantially equimolecular quantities, or with as much as 10% excess either way. Reaction temperatures range from about 129° C. up to about 190° C., dependent upon the nature of the particular reactants. The dihydroxyalkylamide obtained is usually a waxy-solid

product varying in color from white to yellow, light-tan or brown.

The dihydroxyalkylamide may, if desired, be condensed with ethylene oxide, or an equivalent thereof, in the presence of a catalyst, such as sodium hydroxide, to form a polyglycolamide derivative which may be used in further reactions in somewhat similar fashion to the dihydroxyalkylamide. The dihydroxyalkylamide and the ethylene oxide may be condensed in various molar proportions up to as high as 1:50 or even 1:100 or more, but a ratio of approximately 1:6 has been found preferable when textile agents are desired.

These polyglycolamide derivatives may be polyesterified by heating for a long enough time at a proper pressure with maleic anhydride, or its equivalent, and then sulfonated to yield products having the following polymeric formula (when the initial reactants were a fatty acid and diethanolamine):



25 wherein  $M_e$  is a salt-forming cation derived from any of the alkali metals, ammonium or other bases;  $R_1$  is the alkyl or alkenyl radical of a fatty acid;  $n$  is the degree of polymerization, as measured and determined by the acid number; and  $x$  and  $y$  are integers with their sum being as high as 100.

30 In the case where the dihydroxyalkylamide is derived from the reaction between a fatty acid and diethanolamine and is not condensed with ethylene oxide, the resulting product, when polyesterified with maleic anhydride and then sulfonated, possesses the following gen-



40 wherein  $R_1$ ,  $M_e$  and  $n$  have meanings as previously stated.

The invention will be further illustrated in greater detail by the following specific examples. It should be understood, however, that although these examples may describe in particular detail some of the more specific features of the present invention they are given primarily for purposes of illustration and the invention in its broader aspects is not to be construed as limited thereto.

### EXAMPLE I

The preparation of the polysulfosuccinate ester of diethanolstearamide involved three steps. First, diethanolstearamide (*N,N*-bis-(2-hydroxyethyl) stearamide) is made by reacting stearic acid with diethanolamine. In step two, the diethanolstearamide is esterified with maleic anhydride in order to derive the polymeric alkyd. In step three, this alkyd is then sulfonated with sodium bisulfite to yield the desired polysulfosuccinate ester.

### Step I—Preparation of diethanolstearamide



65 239 grams (0.85 mole) of stearic acid was reacted with 101 grams (0.94 mole) of diethanolamine at temperatures of approximately 154-184° C. under an inert atmosphere of carbon dioxide. The temperature was held within the above-indicated range for about 2.3 hours  
 70 and approximately 23.0 ml. of water were collected during that time in a "Barrett" moisture collector. Approximately 8.7% of the diethanolamine remained unreacted. The diethanolstearamide itself was a light cream wax. After completion of the reaction, a titration showed the presence of approximately 5.0% basic impurities which  
 75

may be removed by washing the diethanolstearamide with an acid such as hydrochloric or the like, followed by a neutralization with sodium carbonate. A yield of 172 grams (52%) was determined. The final product was a white solid wax.

In another instance, the preparation of the diethanolstearamide was carried out in the presence of an inert solvent, such as xylene, at a temperature of 130-150° C. The developed water was collected in a "Barrett" moisture collector during the reaction which required between 6 to 16 hours, at the end of which time 4.5 to 7.0% basic impurities were present. The impurities were removed as above-described and the rest of the preparation continued as described below.

*Step II (A)—The preparation of the polymaleate of diethanolstearamide*



The polymaleate of diethanolstearamide is prepared by



esterifying the diethanolstearamide with maleic anhydride or its equivalent. A p-toluenesulfonic acid catalyst may be employed and the esterification may take place, if desired, in the presence of an inert solvent such as xylene, but better results have occasionally been obtained without such additions.

172 grams (0.46 mole in 5% excess) of diethanolstearamide and 46.4 grams (0.48 mole) of maleic anhydride were charged into a one-liter flask equipped with a stirrer, condenser with water trap, and thermometer and refluxed at 165-180° C. under an inert atmosphere of carbon dioxide. 2.0 ml. water were collected in the "Barrett" moisture collector during the 10-hour reaction time. A chain length of 4.2 units was indicated by the acid number which was 28.2. The product was a dark-brown wax obtained in the amount of 182 grams (84% yield).

The preceding esterification was also carried out in the presence of an inert solvent such as toluene (150 ml.) and 5.0 grams of p-toluenesulfonic acid catalyst and the refluxing temperature was held at 125° C. for 23 hours. The chain length of the sample at the end of that time was 2.5 units. The toluene was distilled off under vacuum. The product was a tan wax obtained in 100% yield. When xylene was used as the inert solvent, the chain length was approximately 2.7 units.

*Step II (B).—Preparation of the polymaleate of the diethanolstearamide-ethylene oxide condensation product*

A condensation product of diethanolstearamide and ethylene oxide was prepared as an alternative compound to the diethanolstearamide to be used in the later preparation of the polysulfosuccinic esters. The following procedure was used:

Materials used:

Diethanolstearamide—156.5 grams (0.42 mole).  
Sodium hydroxide—2.1 grams.  
Ethylene oxide—112. grams (2.53 moles).

The stearamide and the sodium hydroxide catalyst were charged into a flask equipped with a stirrer, ice-cooled condenser, thermometer and gas inlet. Ethylene oxide

was passed through a trap into the reaction mixture held at a temperature of 120-130° C. The condensation of the ethylene oxide was slow at first, but proceeded more readily after a few moles of ethylene oxide had been added. The sodium hydroxide catalyst was neutralized with hydrochloric acid. The amount of ethylene oxide added to the diethanolstearamide was determined by weighing the flask before and after the addition of the gas. The product was a dark brown rubbery wax.

The polymaleate of the diethanolstearamide-ethylene oxide condensate may then be prepared by reacting the condensate with maleic anhydride in substantially equimolecular quantities at 130-165° C. for about 32 to 36 hours under an inert atmosphere of nitrogen. An inert solvent and a catalyst may be employed, if desired. Water was collected, as usual, the chain length was indicated to be 6.4 to 6.7 units by the acid number which was 11.5 to 12.3. The product was a tan to dark-brown brittle wax obtained in approximately 90% yield and was suitable for preparation of the polysulfosuccinate ester as set forth in Step III following.

*Step III.—Sulfonation of the alkyds of diethanolstearamide*



The alkyds of diethanolstearamide (or the diethanolstearamide-ethylene oxide condensation product) were reacted with sodium bisulfite (in 10% excess) in an aqueous alcoholic medium (ethanol). The degree of sulfonation of the polymaleates was followed by an iodine titration. Alkyds of diethanolstearamide with chain lengths of 2.5 units were completely sulfonated at the end of 17-22 hours. The excess bisulfite was oxidized with hydrogen peroxide and the product filtered. The polysulfosuccinates were neutralized to a pH of 6.5 with sodium hydroxide and evaporated to dryness on the steam bath and in a forced draft steam oven or left as a paste. The product was a brittle, tan wax (100%) or a thick, tan paste containing approximately 25% solids.

EXAMPLE 2

*Preparation of the sulfosuccinate polyester of diethanollaurylamine*



Diethanollaurylamine (*N,N*-bis-(2-hydroxyethyl)stearamide) was prepared by refluxing lauric acid with a 1% excess of diethanolamine in xylene until water ceased distilling from the reaction mixture. The xylene was then removed from the amide by distillation under reduced pressure up to a temperature of 150° C.

A mixture of 34.2 g. (0.349 mole) of maleic anhydride, 105 g. (0.349 mole+5% excess) of diethanollaurylamine, 175 ml. of toluene, and 5 g. of p-toluenesulfonic acid was refluxed for seventeen hours at 110-115° C., removing the water formed in a trap. The toluene was distilled off under vacuum, leaving the polymaleate ester as a brown brittle waxy solid. The yield was 131 g., and the ester had an acid number of 37.2 indicating an average chain length of 4.1 ester units.

7

This polyester was mixed with 75.5 g. (0.349 mole + 10% excess) of sodium metabisulfite, 200 ml. of ethanol, and 200 ml. of water, and the mixture was refluxed with agitation for twenty-eight hours. It was treated with sufficient 30% hydrogen peroxide to oxidize the excess bisulfite, stirred with "Hyflo," and filtered. The pH was adjusted to approximately 6.5 with sodium hydroxide and the solution was evaporated on the steam bath. After drying at 100° C. the product was obtained as a brown mass. The yield was 131 g.

### EXAMPLE 3

### *Preparation of the sulfosuccinate polyester of diethanolstearamide*



A solution of 157.5 g. (0.404 mole + 5% excess) of diethanolstearamide (prepared by the same procedure used for diethanolauramide), 39.6 g. (0.404 mole) of maleic anhydride, and 5 g. of p-toluenesulfonic acid in 150 ml. of toluene was refluxed at 120-125° C. for twenty-four hours. After the first twenty hours, 65% of the theoretical amount of water was collected in the trap and no more distilled out. After distilling off the toluene under reduced pressure, titration of a sample of the maleate polyester indicated an average chain length of 2.5 ester units. The yield was 196 g. of brown wax.

This polyester, 192 g. (0.426 mole), was mixed with 87 g. (0.457 mole) of sodium metabisulfite, 200 ml. of ethanol and 200 ml. of water and the mixture was refluxed with agitation for twenty-two hours. Iodometric titration of the excess bisulfite indicated the sulfonation was complete. Another 200 ml. of water and 100 ml. of ethanol was added and the excess bisulfite was oxidized with hydrogen peroxide. On cooling, it formed a light tan paste containing 24% solids.

**EXAMPLE 4**

The following example illustrates the use of 2,3-dihydroxypropylamine and stearic acid in the preparation of the polyester of sulfosuccinic acid:

*Step I.—Preparation of the dihydroxyalkylamide*



The equipment comprised a 500 ml., 3-neck flask, equipped with a thermometer, nitrogen inlet tube, stirrer, water trap and condenser. The reactants were heated at 180–205° C. for approximately 10 hours with nitrogen bubbling through the mixture, during which time 28 mls. of water were distilled off. A titration of the product indicated that there was no free acid or base.

8

**Step II.—Polyesterification of the dihydroxyalkylamide**



| [Product from Step I (1-stearamido 2,3-propanediol)] |              |          |       |
|------------------------------------------------------|--------------|----------|-------|
| 15                                                   | Fumaric acid | 0.5 mole | 58 g. |
|                                                      | Xylene       | 85 mls.  |       |

The equipment comprised a 500 ml., 3-neck flask, equipped with a thermometer, nitrogen inlet tube, stirrer, water trap and condenser. The reactants were refluxed for approximately 3 hours in which time a gel was formed. 12 mls. of water were distilled off during this reaction. Titration gave an acid number of 17 and a value for "n" of 7.4.

#### Step II.—Sulphonation of the polyester



## REACTANTS

Na<sub>2</sub>SO<sub>3</sub> 6.3 g (98% pure)

Na<sub>2</sub>SO<sub>3</sub>, 6.5 g. (

Na<sub>2</sub>S<sub>3</sub>O<sub>5</sub>, 28.0 g.  
160 mls. benzene

100 mls. benzene  
150 mls. alcohol

150 mls. water

45 The equipment comprised a 1-liter, 3-neck flask equipped with a stirrer, thermometer and reflux condenser. The reactants were refluxed on a steam bath for about 13 hours at approximately 65° C. 250 mls. of solvent was stripped to raise the reflux temperature  
50 to approximately 75° C. and then 250 mls. of a 1:1 mixture of alcohol and water added.

The reaction mixture was then refluxed for approximately 14 more hours (or 27 hours total) and 250 mls. alcohol was added. After a total of 62 hours of refluxing, 48% sulfonation by titration was indicated. The unreacted bisulfite was oxidized to bisulfate with 235 mls. of 30%  $H_2O_2$  and the bisulfate was neutralized to sulfate with 25% NaOH. The product was diluted with 500 mls. alcohol and 500 mls. benzene; "Hyflo" was added and the product was filtered by suction. The filtrate was then evaporated on a steam bath.

In employing the novel polyesters of the invention in textile softening treatments, a dispersion from about 0.25% to about 3% or more of the selected polyester is prepared in a water bath or, if the textile is to be sized at the same time, in an aqueous size bath. The textile material is thereafter impregnated in the bath up to a wet pickup of substantially 100% of the weight of fabric and then dried according to normal operating procedures. Ordinarily, where no sizing agent is employed, it is unnecessary to have more than about 1% of the softening agent on the fabric in order to obtain the desired softness of hand in the product. On the other hand, where a sizing agent is used, it is sometimes necessary to increase the softening agent content to about 3% or more

to obtain the desired improvement in softness of hand in the treated fabric.

Testing of the non-yellowing softening agents of the present invention revealed that they possessed the following advantages. No serious yellowing was produced in fabrics when they were heated at 95° C. for three days. The use of these agents did not cause any shade changes nor did they decrease the light fastness of dyes on the tested fabrics. These agents were easily dispersible liquids or pastes and were further found to soften or plasticize starch finishes.

Other uses for the novel compounds of the present invention would include emulsifying agents for any purpose, such as the lubrication of textile materials with mineral oils; fat-liquoring of leather; preparation of insecticidal sprays; emulsion polymerization processes; detergents; flotation of ores and minerals; dispersing agents, e. g. or pigments; demulsifying agents; scouring of wool; dyeing assistants; softening of paper hand towels; etc.

Although I have described but a few specific examples 20 of my inventive concept, I consider the same not to be limited thereby nor to the specific substances mentioned therein, but to include various other compounds of equivalent constitution as set forth in the claims appended hereto. It is to be understood, of course, that any suitable changes, modifications and variations may be made without departing from the scope and spirit of the invention.

I claim:

1. A method of softening textile material which com- 30

prises impregnating the textile material with an aqueous dispersion of a polymeric sulfosuccinate ester of a fatty acid dihydroxyalkylamide, said ester having at least two but not more than about twelve ester units and said fatty acid containing more than 7 carbon atoms.

2. A method as defined in claim 1 in which the aqueous dispersion contains from about 0.25% to about 3% by weight of the polymeric ester.

3. A method as defined in claim 2 in which the pick-up of aqueous dispersion by the textile material is substantially 100% of the weight of the fabric.

4. A textile material characterized by improved softness of hand and having distributed therethrough from about 0.25% to about 3% by weight of a polymeric sulfosuccinate ester of a fatty acid dihydroxyalkylamide, said polymeric ester having at least two but not more than about twelve ester units and said fatty acid containing more than 7 carbon atoms.

#### References Cited in the file of this patent

#### UNITED STATES PATENTS

|           |                      |              |
|-----------|----------------------|--------------|
| 2,002,613 | Orthner et al. ----- | May 28, 1935 |
| 2,236,528 | Epstein et al. ----- | Apr. 1, 1941 |
| 2,637,663 | Thurston -----       | May 5, 1953  |

#### OTHER REFERENCES

Chemical Abstracts, 31:1359, D'Alelio et al., Three Series of N-substituted Aliphatic Amides.